

Nov. 6, 1951

A. C. SCAVULLO

2,573,736

METHOD OF MAKING HOLLOW ARTICLES

Filed Feb. 24, 1947



## UNITED STATES PATENT OFFICE

2,573,736

## METHOD OF MAKING HOLLOW ARTICLES

Angelo C. Scavullo, Forest Hills, N. Y., assignor to  
Victor K. Scavullo, Frank Scavullo, Charles  
Scavullo, Marie Scavullo Saegert, and Margaret  
Scavullo Scott, all of Forest Hills, N. Y.

Application February 24, 1947, Serial No. 730,451

2 Claims. (Cl. 29—148.2)

1

My invention relates to fabricated metal products, more especially to hollow-ware articles and to a method for producing the same.

An object of my invention is the provision of a simple, direct and thoroughly reliable method for fabricating ornamented and integrally reinforced articles of the character described from stainless steel sheet, wherein the ornamentation and reinforcement are readily achieved during the fabricating operations.

A further object of my invention is the provision of simply and economically produced stainless steel hollow-ware articles which are strong, durable and easy to keep in thoroughly presentable and attractive condition even when put to hard usage.

Other objects of the invention in part will be obvious and in part pointed out hereinafter.

The invention accordingly consists in the features of construction and in the several operational steps, and the relation of each of the same to one or more of the others as described herein, the scope of the application of which is indicated in the following claims.

For a more ready comprehension of an embodiment of my invention, reference may be had to the accompanying drawing, wherein:

Figure 1 is a perspective view of a preliminarily formed hollow-ware article;

Figures 2 and 3 are views illustrating certain forming operations in accordance with my invention; and

Figures 4 and 5 are detached sectional views of two forms of the hollow-ware article of my invention.

Like reference characters denote like parts throughout the several views.

As conducive to a clearer understanding of certain features of my invention, it may be noted at this point that stainless steels, as for example the austenitic chromium-nickel stainless steels and especially those containing 10% to 25% chromium and 7% to 15% nickel, and the remainder substantially all iron, have come into widespread use in a number of interior and exterior architectural applications, such as decorative trim and fixtures, where bright metal resistant to the corrosive effects of atmospheric conditions is advantageous. Likewise, the straight-chromium stainless steels, as for example those containing from 12% to 18% chromium and the remainder substantially all iron have been employed for similar uses.

In recent years the stainless steels have been extensively in demand for a variety of kitchen,

dairy and hospital applications, as in the form of cooking and serving utensils exposed to fruit and vegetable acids or corrosive salts, common containers, and other appliances where bright corrosion-resistant metal is desired. This and other demands have made it desirable to produce stainless steel hollow-ware articles, as for example bric-a-brac, bowls, gravy boats, coasters, ladles, dishes, pitchers, pots, trays, and the like, in competition with similar articles made of plain carbon steel or silver. A selling point in favor of stainless steel products, illustratively hollow-ware table settings, is their pleasing, rich and enduring surface appearance whether they be bright polished or left in their satin-like gray unpolished condition. The stainless steel commodities further present the attraction of being economical to use, for such reasons as having a relatively low initial cost as compared with articles made of precious metals, and of being extremely durable and requiring little maintenance and infrequent replacement even under conditions of hard usage.

As distinguished from conventional stainless steel hollow-ware, I find ornamentation desirable. The provision of stainless steel products in ornamented form in which the utilitarian aspects of the steel are substantially fully retained, may therefore be regarded as an outstanding object of my invention. Another object is the production of such ornamented articles at minimum cost.

Referring now more particularly to the practice of my invention, I produce ornamental stainless steel hollow-ware, as for example any of a wide variety of pieces for table use, by first forming hollowed or dished articles from stainless steel sheet or strip as by stamping, bending or deep-drawing. I provide an ornamental brim or lip on the ware, by such measures as rolling, pressing, bending or spinning the free edge of the sheet or strip thus achieving a turned-over welded thickness or overlapping border.

While the articles of my invention may be formed having merely a plain border for the ornamental effect, I usually provide further ornamentation, this illustratively being raised or impressed designs on the portion constituting the border. For this purpose I employ cooperating dies, the latter advantageously being applied bearing toward each other across the thickness of the stainless steel at a pressure which is so moderate that the metal surface in being decorated takes a sharp impression without detrimental distortion or undue weakening of the article. The dies for example are roller dies, one constituting a raised die and the other having a

corresponding depressed pattern cut therein. As an alternative, one of the dies may be entirely smooth to afford a back-up for the other an ornamentation-imparting die which supports a pattern in the form of an intaglio or raised areas producing the stainless steel surface decoration. There are occasions when I apply ornamentation to the single thickness of the metal without later turning down the brim or lip, but otherwise enjoy the benefits derived from working and ornamenting the metal.

The stainless steel hollow-ware articles which I produce have any of a variety of different shapes and sizes, as in the instance of plates, platters, trays, coffee pots, urns, tumblers, vases, pans, dishes and numerous other products. In general the stainless steel sheets from which I fabricate the articles have gauge thicknesses ranging between 12 to 20 gauge or less. Where the articles are to have an overlapping border I find advantage in using thin sheets of the steel, preferably from 18 to 20 gauge sheets and even smaller gauges. With the overlapping border at the brim or lip, my hollow-ware articles are especially strong and capable of withstanding rough usage commonly encountered in restaurants, hotels and the like. Moreover, the border or overlapping rim greatly contributes to overall decorative effect, particularly where this effect is enhanced by embossed or stamped designs on the rim or on other areas of the ware. Both the rim and the remainder of the stainless steel products resist corrosion, this also being true of any designs which I cut or press on the metal by dies or the like.

As specifically illustrative of the practice of my invention, I deep-draw 18 gauge stainless steel sheet into the preliminary form of a particular article of stainless steel, as for example into the rough form of a salad bowl 10 represented by Fig. 1 of the accompanying drawing. The preliminary fabricated bowl has a flat out-turned marginal rim 10a, this conveniently being produced as an incident to the deep-drawing operations and thereafter trimmed to desired width by any suitable metal cutting tool or machine. While the article may be fabricated from any suitable stainless steel, I find that 18-8 chromium-nickel steel (18% chromium, 8% nickel and the remainder substantially all iron) serves admirably for the purpose.

For providing a pressed-in ornamental design or intaglio on the rim 10a, I employ co-operating rotary dies, one of these (see Fig. 2) being an overlying circular rotary die element 11 fast on drive shaft 11a through its hub 11b. On the peripheral face 11c of the element there is a male die pattern 11d which serves to cut the ornamental design or intaglio into the top surface of the rim 10a. Beneath the roller 11, is a cooperating circular and rotary die element 15 having a smooth peripheral surface 15c affording a back-up or anvil surface for the male die pattern 11. The die element 15, for example is loosely mounted as an idler on shaft 15a, or is driven by the shaft through a positive connection of the hub 15b.

With the rotary die elements disposed a suitable distance apart, I introduce the rim 10a of the salad bowl between the same, and then adjust the dies to cutting position of the pattern 11d against the rim. Then, by rotating the dies, as by driving the respective shafts 11a and 15a in opposite and aiding directions of rotation, and at the same feeding rate, a feeding and pressing

action comes into play on the rim 10a. The rate of speed of the rim and the pressure exerted thereon, as achieved by the die elements, are sufficient that the rim top surface takes a good, sharp impression or intaglio of the male pattern 11d. The effect of this impression is executed by the back-up die from the directly opposing surface of the sheet metal thickness. I maintain the working conditions until the pattern defines a closed path on the rim and impresses the circuitous ornamental design 10b in the stainless steel surface. Where desired, I cut or emboss other ornamentation on the surface of the bowl, apart from the rim surface, as in a circuit around the outside area of the concave stainless steel body and by employing the same or similar dies as are used in decorating the rim. Where the back-up die element 15, however, is to contact surfaces of the ware which are to be exposed to view, I find advantage in padding the element so as to avoid imparting injurious scars and scratches by the same during the pressing or cutting of the stainless steel.

In finishing the deep-drawn bowl, I subject the rim to bending operations such as to produce a flat, compact outside or inside border of the same (see Figs. 4 and 5) at the brim of the ware. The bending operations preferably include spinning to expedite production and for satisfactorily avoiding defacement of the ornamented rim. For spinning, I support the stainless steel bowl illustratively between rotary clamping plates 20, 21, as represented in Fig. 3. These plates are suited for simultaneous rotation by their aligned axial shafts 20a, 21a, and as a unit with the bowl. To advantage, I back-up the bowl in the vicinity of the brim, for example by use of an inside roller 22, mounted as for idling movement on the supporting shaft 22a and held to adjusted bearing position against the inner bowl surface by suitable means not shown. Also, in the present instance, I use an outside roller, or quadrant roller 23 (conveniently journaled in a forked carrier 23a and operative by gradually tilting through about 90° with the carrier), so as to turn the ornamented rim 10a flat against the main body of the bowl while the latter is backed up by the inside roller 22 and rotated by the plates 20 and 21.

During the last stages of these spinning operations I introduce molten solder into the space 10c, as a beneficial practice, and press the rim 10a to soldered relation with the adjoining stainless steel surface of the ware. The solder-filled overlap accordingly is held firm, and well closed off against contamination by such materials as foods, dirt, and the like, which otherwise might lodge in the space 10c. The salad bowl is highly satisfactory for use either in the natural unpolished condition or after bright polishing as by a light electrolyte polishing treatment or by mechanical polishing methods, as desired. It will be appreciated that the topmost portion or lip of the bowl has a continuous, corrosion-resistant stainless steel surface which is easy to keep free of corrosion and clean during use of the ware. The ornamental design or intaglio 10b extends in full view all way around the border.

In carrying out my process, it therefore is possible to provide a pleasing, clear and substantially undistorted ornamental touch such as beading, gadrooning or edging on stainless steel hollow-ware, and the like, and this in a rapid, certain manner. The neat, integral border on the ware, whether decorated or plain, is readily

produced and lends structural reinforcement and artistic appeal. As has been suggested, stainless steel hollow-ware, and generally similar articles made in accordance with my invention, have pleasing appearance and substantial sales attraction, the price differential as compared with the cost of articles formed of precious metals such as silver adding appreciably to marketability and attractiveness to the discriminating pur-chaser.

It must also be noted that my process has utility for continuous production by proper co-ordination and arrangement of the equipment employed in effecting the several steps, and may be satisfactorily practiced with reliance upon labor of moderate skill in maintaining low cost and high utility of the hollow-ware products achieved.

Thus it will be seen that there is provided in this invention a production process for making stainless steel hollow-ware articles, and products of the process, in which the various objects hereinbefore noted together with many thoroughly practical advantages are successfully achieved. It will be seen that the process and products are representative of satisfactory and economical production in a highly competitive field.

While the stainless steel hollow-ware articles produced in accordance with my invention may be either in the natural gray metallic or bright polished surface condition, it will be appreciated that at times the articles are given other surface finishes such as by blackening treatment following production to desired final shape.

It will be understood that I apply my process to producing nickel or copper hollow-ware articles, as for example articles ornamented and lapped at the brim, from approximately 12 to 20 gauge sheet nickel or copper, with certain of the advantages had with stainless steel.

As many possible embodiments may be made of my invention, and as many changes may be made in the embodiment hereinbefore set forth, it is to be understood that all matter whether described or illustrated herein is to be interpreted as illustrative and not as a limitation.

I claim as my invention:

1. In the production of sheet metal hollow-ware articles, the art which includes, forming the sheet into desired hollowed configuration with a free edge portion, positioning the hollowed formed sheet between rotary clamping plates, then while backing up the main body of sheet spinning the free edge of sheet to an overlapping border by applying pressure to the free spinning

edge, and introducing molten solder between said border and the main body of said sheet during final stages of the spinning operation.

2. In the production of ornamented stainless steel, nickel or copper hollow-ware articles, the art which includes, shaping sheet of the metal to desired article configuration with body portion and free edge portion, passing said free edge portion of said sheet continuously between a rotary smooth surfaced anvil die and a cooperating rotary ornamentation-imparting die for producing a surface decoration thereon, backing up the body portion with an inside roller and spinning the free edge portion into an overlapping border with exposed surface decoration, and during the spinning operation introducing solder between the border and the body portion of the article.

ANGELO C. SCAVULLO.

#### REFERENCES CITED

The following references are of record in the file of this patent:

#### UNITED STATES PATENTS

| Number    | Name            | Date           |
|-----------|-----------------|----------------|
| 145,334   | Cass            | Dec. 9, 1873   |
| 145,400   | Cole            | Dec. 9, 1873   |
| 203,328   | Edgar           | May 7, 1878    |
| 425,809   | Leach           | Apr. 15, 1890  |
| 426,407   | Browning        | Apr. 22, 1890  |
| 464,385   | Palmer          | Dec. 1, 1891   |
| 699,795   | Eynon           | May 13, 1902   |
| 761,792   | Such et al.     | June 7, 1904   |
| 1,374,225 | Peacock         | Apr. 12, 1921  |
| 1,552,017 | Sturges         | Sept. 1, 1925  |
| 1,572,492 | Kemper          | Feb. 9, 1926   |
| 1,717,482 | Weidlich et al. | June 18, 1929  |
| 1,718,322 | Walker          | June 25, 1929  |
| 1,728,033 | Blake et al.    | Sept. 10, 1929 |
| 1,785,905 | Kerruish        | Dec. 23, 1930  |
| 1,807,141 | Wood            | May 26, 1931   |
| 1,966,713 | Flint           | July 17, 1934  |
| 1,981,915 | Hormel et al.   | Nov. 27, 1934  |
| 2,006,894 | Hulbert et al.  | July 2, 1935   |
| 2,040,102 | Peron           | May 12, 1936   |
| 2,057,254 | Sommer          | Oct. 13, 1936  |
| 2,083,440 | Fink            | June 8, 1937   |
| 2,125,793 | Linderman, Jr.  | Aug. 2, 1938   |
| 2,132,796 | Money           | Oct. 11, 1938  |
| 2,310,834 | Bullock         | Feb. 9, 1943   |

#### FOREIGN PATENTS

| Number  | Country       | Date          |
|---------|---------------|---------------|
| 444,565 | Great Britain | Mar. 23, 1936 |